

# UNITED STATES PATENT OFFICE.

DAVID BELAIS AND ALFRED R. BONDY, OF NEW YORK, N. Y.; SAID BONDY ASSIGNOR  
TO SAID BELAIS.

## WHITE GOLD.

1,391,449.

Specification of Letters Patent. Patented Sept. 20, 1921.

No Drawing.

Application filed October 24, 1919. Serial No. 333,067.

To all whom it may concern:

Be it known that we, DAVID BELAIS and ALFRED R. BONDY, citizens of the United States, and residents of New York, in the county and State of New York, have invented a certain new and useful Improvement in White Gold, of which the following is a specification.

Our invention relates to the production of an improved white gold. It is an improvement upon the white gold composition set forth in the patent of David Belais, one of the applicants herein, No. 1330231 of Feb. 10, 1920, which composition consisted of an alloy of gold, nickel and zinc. Like the white gold described in the said patent, our improved alloy has the appearance of platinum, and may be used as a substitute for it, especially in the jewelry art. It is tenacious, and is much more ductile and malleable than the white gold of said patent, and is adapted for certain uses for which the said white gold is unfitted. For example, while the white gold of said patent can be drawn into solid wire, it is impossible to draw it into tubing, or seamless tubing. Our improved alloy, because of its highly tenacious, ductile and malleable character, can not only be drawn into solid wire, but can be drawn into tubing such as seamless tubing. This fits it for uses to which the said white gold, and all other white golds on the market, are unadapted.

In the production of our improved alloy we take gold, especially or preferably fine gold, nickel, preferably pure nickel, zinc, preferably pure zinc, and a minute quantity of platinum, and fuse them together in a suitable crucible, thoroughly mixing them together while they are thus fused. The resulting composition has the appearance of platinum and has the characteristics, and is adapted for the uses, above described. The alloy is prepared for the market in any suitable manner and form. We use a major part of gold and lesser parts of nickel and zinc, the zinc being used preferably in lesser proportions than the nickel, and the platinum being used in relatively minute quantities, less than one per cent. and preferably less than one-half of one per cent. We have

found that satisfactory results can be obtained when the gold is used in the proportion of about seventy-five (75) to eighty-five (85) per cent., nickel in the proportion of about ten (10) to eighteen (18) per cent., zinc in the proportion of about two (2) to nine (9) per cent., and of platinum only a fraction of a per cent., less than one-half ( $\frac{1}{2}$ ) per cent., and preferably from one-thirtieth (1/30) or one-twenty-fifth (1/25) to one-half ( $\frac{1}{2}$ ) of one per cent.

What we claim as new and desire to secure by Letters Patent, is:

1. As a composition of matter, a white gold alloy composed of a major part of gold, lesser proportions of nickel and zinc, and a minute quantity of platinum adapted to make the alloy sufficiently ductile to be drawn into seamless tubing.

2. As a composition of matter, a white gold alloy composed of a major part of gold, a lesser proportion of nickel, a still lesser proportion of zinc, and a minute quantity of platinum adapted to make the alloy sufficiently ductile to be drawn into seamless tubing.

3. As a composition of matter, a white gold alloy composed of gold, nickel, zinc and platinum, the proportion of gold running from seventy-five (75) to eighty-five (85) per cent., the nickel from ten (10) to eighteen (18) per cent., the zinc from two (2) to nine (9) per cent., and the platinum being sufficient in amount to be adapted to make the alloy ductile enough to be drawn into seamless tubing but not exceeding one-half of one per cent.

4. As a composition of matter, a white gold alloy composed of gold, nickel, zinc and platinum, the proportion of gold running from seventy-five (75) to eighty-five (85) per cent., the nickel from ten (10) to eighteen (18) per cent., the zinc from two (2) to nine (9) per cent., and the platinum from one-thirtieth to one per cent. to one-half of one per cent.

In testimony whereof, we have signed our names to this specification.

DAVID BELAIS.  
ALFRED R. BONDY.